

1

3,511,660

**ANTIHALATION BACKING FOR PHOTOGRAPHIC SILVER HALIDE RECORDING ELEMENTS**  
Guy William Willis Stevens, Harrow, England, and Claude Masson, Vincennes, France, assignor to Eastman Kodak Company, Rochester, N.Y., a corporation of New Jersey  
No Drawing. Filed Oct. 18, 1966, Ser. No. 587,398  
Claims priority, application Great Britain, Oct. 19, 1965, 44,276/65; France, Dec. 1, 1965, 40,414  
Int. Cl. G03c 1/84

U.S. Cl. 96—84

8 Claims

### ABSTRACT OF THE DISCLOSURE

A photographic element comprises a support having on one side a photosensitive layer such as a silver halide emulsion and on the other side an antihalation layer comprising carbon black in a binder such as cellulose acetate phthalate and having colloidal silver in the antihalation layer. The colloidal silver inhibits fading, etc., caused by carbon black contacting the silver halide in film rolls and the like.

The present invention relates to sensitive photographic materials, especially sensitive silver halide coated films having backing layers.

When sensitive photographic films which have layers coated on the rear side of the support are packed so that the rear side of one piece of film presses in contact with the front sensitive side of another piece, problems sometimes arise caused by undesirable effects produced on storing the films so packed, where substances present in the backing layer adversely affect the sensitive layers. This kind of trouble can sometimes be very serious in the case of rolls of films because in almost every convolution of the roll, some part of the rear surface is pressing against the front surface of the next convolution.

Of the many substances which have been suggested for making light absorbing and antihalation layers, carbon black is especially suitable. However, we have found that most, if not all, available commercial carbon black, when incorporated in the backing layer of sensitive films, especially films bearing on their front surface a highly sensitive gelatino-silver halide emulsion layer, produce undesirable effects of the kind referred to, especially when the film is stored for long periods in rolls in climates of rather high humidity. In the case of this carbon black the effect may be particularly serious when the silver halide layer has been exposed imagewise and therefore contains a latent image. On storage of such exposed film in high humidity conditions, the carbon black produces an undesirable fading of the latent image and of course this fading is usually not uniform but varies area by area according to the tightness of the contact in the convolutions of the roll.

Since the reason why some carbon black produces this undesirable effect even when in a binder, such as cellulose acetate phthalate is obscure, it has been extremely difficult to overcome. We have now found however, that the effect can be eliminated or reduced to such a low degree as to be insignificant, by incorporating colloidal silver in the layer containing the carbon black or by coating over the carbon black layer a separate layer containing the colloidal silver.

For simplicity of manufacture, it is preferred that the colloidal silver be added to the coating solution used for coating the carbon black layer. While small propor-

2

tions of colloidal silver to carbon can be usually added without difficulty, there is a tendency in the case of many vehicles, especially the organic solvent soluble vehicles such as cellulose acetate phthalate, for the carbon and silver to flocculate each other, especially in cases where the carbon black is itself in a state of incipient flocculation. In order therefore to incorporate larger and more useful quantities of colloidal silver without flocculation of either the silver or the carbon occurring, we have found that the following procedure should be adopted.

(A) Disperse the carbon black in a solution of the binder, such as cellulose acetate phthalate, using as solvent a mixture of water with a water-miscible organic liquid which is itself a solvent for the binder.

(B) Make a dispersion of colloidal silver in a mixture of water with a water-miscible organic liquid which is itself a solvent for the binder used for (A).

These two dispersions (A) and (B) are then simply mixed together with stirring.

This method permits the incorporation of colloidal silver to the dispersion of carbon black in the solvent medium containing the cellulosic binder, used for coating the antihalation backing layer.

It is also possible to disperse beforehand the colloidal silver in the cellulose binder in a solvent medium and to add this preparation to the carbon black dispersion.

The quantities to be added are such that the silver to carbon ratio by weight may vary from 1 to 100 to 1 to 2 but we prefer to use quantities between 1 to 30 and 1 to 4 of silver having the particle size described herein. The important property of the silver is its particle size so that using smaller particle sizes allows the weight to be reduced and vice versa.

For incorporating the colloidal silver by this method, the carbon black is first completely dispersed in a solvent medium of the cellulose binder (A), then diluted with a mixture which is equally a solvent, of the cellulose binder, but containing a dispersion of colloidal silver in an aqueous medium (B).

The following examples illustrate the invention.

### EXAMPLE 1

Twenty-five grams of polyvinyl phthalate (19% phthalyl) are dispersed in the following mixture:

|                                 | Ml. |
|---------------------------------|-----|
| Ethylene glycolmonomethyl ether | 140 |
| Ethanol                         | 90  |
| Water                           | 30  |

To the dispersion so made there is then added the following dispersion of colloidal silver:

|                                                        | Ml. |
|--------------------------------------------------------|-----|
| Ethylene glycolmonomethyl ether                        | 120 |
| Ethanol                                                | 376 |
| Acetone                                                | 123 |
| 12.5% by weight "Codex"-type colloidal silver in water | 120 |

"Codex"-type colloidal silver is pharmaceutical colloidal silver conforming with the "Codex" of the Pharmacie Francais; it must disperse spontaneously in water and contain not less than 68 percent of silver combined with protein. The silver particles have a diameter of about 10 to 12 millimicrons.

The resulting silver dispersion is very stable.

Eighty ml. of this dispersion are added with stirring to 1000 ml. of a dispersion of carbon black in cellulose acetate hexahydro phthalate prepared in the following way.

## 3

Forty-two grams of a solid dispersion comprising  $\frac{1}{3}$  of carbon black in  $\frac{2}{3}$  of cellulose acetate hexahydro phthalate are dissolved in:

|                                 | ML. |
|---------------------------------|-----|
| Ethylene glycolmonomethyl ether | 150 |
| Ethanol                         | 300 |
| Acetone                         | 63  |
| Water                           | 75  |

The carbon black particles had a diameter of about 30 millimicrons. After dissolution, the following mixture is added with stirring:

|                                 | ML. |
|---------------------------------|-----|
| Ethylene glycolmonomethyl ether | 110 |
| Ethanol                         | 166 |
| Acetone                         | 60  |
| Water                           | 75  |

## 4

After dissolution, there was added with agitation the following mixture:

|                                                                   | ML. |
|-------------------------------------------------------------------|-----|
| Ethylene glycolmonomethyl ether                                   | 110 |
| Ethanol                                                           | 166 |
| Acetone                                                           | 60  |
| Water                                                             | 55  |
| 7.5% solution of "Codex" pharmaceutical colloidal silver in water | 20  |

The coating produced from this backing of silver/carbon ratio 1:9 and a control coated with no silver addition were tested by the procedure described in Example 1.

| Test conditions                   | Density values  |              |            |                     |              |            |
|-----------------------------------|-----------------|--------------|------------|---------------------|--------------|------------|
|                                   | Control backing |              |            | Backing with silver |              |            |
|                                   | Control area    | Contact area | Difference | Control area        | Contact area | Difference |
| 70% R.H. 3 days<br>at 105° F----- | 1.10            | 1.24         | +0.14      | 1.05                | 1.08         | +0.03      |

The resulting mixed dispersion, which has a 1:12 silver/carbon ratio and is very stable, is coated on the back of film base to give a layer containing 15-20 mg. of silver per square meter. The resistivity of the layer is not higher than  $0.20 \times 10^9 \Omega/\text{cm.}/\text{cm.}$

This layer and a control without the silver addition were tested by contacting with a reversal color film exposed to white light to give a neutral density around 1 after commercial processing. Before contacting, both emulsion-coated and backing-coated films were conditioned to a

Again the backing with silver produced a markedly decreased density and color change.

## EXAMPLE 3

A carbon-black-silver layer was made up exactly as in Example 2, except that cellulose acetate hexahydro phthalate was substituted for the cellulose acetate phthalate.

The coatings produced from this backing and a control coated with no silver addition were tested by the procedure described in Example 1.

| Test conditions                   | Density values  |              |            |                     |              |            |
|-----------------------------------|-----------------|--------------|------------|---------------------|--------------|------------|
|                                   | Control backing |              |            | Backing with silver |              |            |
|                                   | Control area    | Contact area | Difference | Control area        | Contact area | Difference |
| 70% R.H. 3 days<br>at 105° F----- | 0.95            | 1.02         | +0.07      | 0.92                | 0.96         | +0.04      |
| 80% R.H. 3 weeks<br>at 70° F----- | 1.28            | 1.38         | +0.10      | 1.22                | 1.26         | +0.04      |

suitable relative humidity. The backing sample was cut to half-the-width of the exposed film, so that there was always a control area of emulsion which did not contact the backing, when the two conditioned layers were rolled together under tension. The rolled film was hermetically sealed in moisture-proof foil, and stored at an appropriate temperature until processing.

After processing, the affected areas of emulsion always showed a yellow patch, and the magnitude of the changes was measured by reading densities through a blue filter.

The backing with silver produced a much decreased density and color change.

## EXAMPLE 2

Forty-two grams of a solid dispersion comprising  $\frac{1}{3}$  of carbon black in  $\frac{2}{3}$  of cellulose acetate phthalate were dispersed in:

|                                 | ML. |
|---------------------------------|-----|
| Ethylene glycolmonomethyl ether | 150 |
| Ethanol                         | 300 |
| Acetone                         | 63  |
| Water                           | 75  |

55 In both testing conditions, the backing with silver produced significantly smaller density and color changes.

## EXAMPLE 4

60 Thirty grams of "Peerless" carbon black sold by Columbian Carbon Company are added to 1.5 grams of "Codex" colloidal silver dissolved in 250 ml. of a mixture of 1,000 ml. ethylene glycolmonomethyl ether and 100 ml. of water, and the mixture is stirred for 2-3 days, then it is filtered, washed with distilled water and dried at 80° C.

65 Fourteen grams of the dry mixture were then dispersed in 28 grams of cellulose acetate hexahydro phthalate to which was added diethyleneglycol monomethyl ether (methyl Carbitol) (11 grams).

70 Forty-two grams of the resulting dry mixture was then added to:

|                                 | ML. |
|---------------------------------|-----|
| Ethylene glycolmonomethyl ether | 140 |
| Ethanol                         | 90  |
| Water                           | 30  |

To the dispersion there was then added:

|                                 | Ml. |
|---------------------------------|-----|
| Ethylene glycolmonomethyl ether | 120 |
| Ethanol                         | 376 |
| Acetone                         | 123 |
| Water                           | 120 |

The resulting product was then coated to give a layer bearing 5-7 mg. of silver per square meter and having a resistivity of about  $0.20 \times 10^9 \Omega/\text{cm.}/\text{cm.}$

The coatings produced from this backing and from a control with no silver addition were tested by the procedure described in Example 1.

In both tests, the clear overcoated control B produced larger color and density changes than the plain control A. The silver-containing overcoat prevented all color change.

It will be understood that modifications and variations may be made within the scope of the invention as described above and as defined in the following claims.

We claim:

1. In a photographic element comprising a support having on one side a photosensitive layer and on the other side an antihalation backing layer which has dispersed therein carbon black, an improvement wherein said antihalation backing layer contains colloidal silver therein.

| Test conditions            | Density values  |              |            |                     |              |            |
|----------------------------|-----------------|--------------|------------|---------------------|--------------|------------|
|                            | Control backing |              |            | Backing with silver |              |            |
|                            | Control area    | Contact area | Difference | Control area        | Contact area | Difference |
| 70% R.H. 3 days at 105° F. | 0.95            | 1.02         | +0.07      | 0.92                | 0.96         | +0.04      |
| 80% R.H. 3 weeks at 70° F. | 1.28            | 1.38         | +0.10      | 1.21                | 1.23         | +0.02      |

#### EXAMPLE 5

Twelve ml. of a Carey Lea silver sol containing 1.6 percent by weight colloidal silver in 3 percent by weight gelatin at 40° C. was mixed with 15 ml. of water at 40° C. This mixture was then poured slowly with stirring into 47 ml. of a solution containing:

|                                    | Percent by volume |
|------------------------------------|-------------------|
| Methyl Cellosolve                  | 19.4              |
| Acetone                            | 20                |
| Ethyl alcohol                      | 60.6              |
| Cellulose acetate phthalate, grams | 30                |
| Methyl Cellosolve, ml.             | 140               |
| Ethyl alcohol, ml.                 | 90                |
| Water (distilled), ml.             | 30                |

Both the silver and gelatin remained satisfactorily dispersed. The resultant mixture was then poured with rapid stirring in 26 ml. of a solution produced from:

|                                    |     |
|------------------------------------|-----|
| Cellulose acetate phthalate, grams | 30  |
| Methyl Cellosolve, ml.             | 140 |
| Ethyl alcohol, ml.                 | 90  |
| Water (distilled), ml.             | 30  |

The mixture was then coated over a carbon/black coating, such as the control of Example 1. This composite coating was labeled C. As controls were used, the plain carbon backing (A) and the carbon backing supercoated with a similar cellulose acetate phthalate solution without any silver added (B).

The three coatings were tested as in Example 1, with the following results.

|                                     | Control coating A | Coating with clear second layer B | Coating with silver in second layer C |
|-------------------------------------|-------------------|-----------------------------------|---------------------------------------|
| Test at 70% R.H. 3 days at 105° F.: |                   |                                   |                                       |
| Control area                        | 0.95              | 0.94                              | 0.93                                  |
| Contact area                        | 1.03              | 1.06                              | 0.93                                  |
| Difference                          | +0.08             | +0.12                             | 0                                     |
| Test at 80% R.H. 3 weeks at 70° F.: |                   |                                   |                                       |
| Control area                        | 0.94              | 0.99                              | 0.97                                  |
| Contact area                        | 1.12              | 1.30                              | 0.85                                  |
| Difference                          | +0.18             | +0.31                             | *-0.12                                |

\*The density loss shown by this test was caused solely by physical pinholes resulting from backing stripping, and not from chemical photographic action of the backing.

25 2. A photographic element of claim 1 in which the support is film base.

3. A photographic element of claim 1 wherein the ratio of said colloidal silver to said carbon black is in the range from about 1 to 100 to about 1 to 2 parts, by weight.

30 4. A photographic element of claim 3 wherein said ratio of colloidal silver to carbon black is in the range from about 1 to 30 to about 1 to 4 parts, by weight.

5. An element of claim 1 in which said carbon black is dispersed in cellulose acetate phthalate.

6. An element of claim 1 in which said carbon black is dispersed in cellulose acetate hexahydrophthalate.

7. An element of claim 1 in which said carbon black is dispersed in polyvinyl phthalate.

35 8. A photographic element of claim 1 in which said photosensitive layer is a silver halide emulsion.

#### References Cited

##### UNITED STATES PATENTS

|           |         |                   |       |    |
|-----------|---------|-------------------|-------|----|
| 2,694,622 | 11/1954 | Hunter            | 96—84 | XR |
| 3,163,533 | 12/1964 | Derr              | 96—22 | XR |
| 3,247,127 | 4/1966  | Bailey            | 96—84 | XR |
| 2,346,078 | 4/1944  | Nadeau et al.     | 96—84 |    |
| 2,448,507 | 9/1948  | Alles             | 96—84 |    |
| 2,462,534 | 2/1949  | Murray            | 96—84 |    |
| 2,968,582 | 1/1961  | Salminen et al.   | 96—87 |    |
| 3,152,252 | 10/1964 | Wainwright et al. | 96—84 |    |
| 3,222,178 | 12/1965 | Nadeau et al.     | 96—87 | XR |
| 3,234,023 | 2/1966  | De Ramaix et al.  | 96—84 |    |
| 3,269,252 | 8/1966  | De Keyser et al.  | 96—84 |    |
| 3,340,062 | 9/1967  | Hunter et al.     | 96—84 |    |

##### FOREIGN PATENTS

|         |         |                |
|---------|---------|----------------|
| 583,508 | 12/1946 | Great Britain. |
|---------|---------|----------------|

RONALD H. SMITH, Primary Examiner

U.S. Cl. X.R.